

F. C. W. TIMM.

PROCESS FOR RECOVERING ZINC FROM ZINKIFEROUS MATERIALS.

APPLICATION FILED OCT. 7, 1913. RENEWED DEC. 31, 1915.

1,172,321.

Patented Feb. 22, 1916.



WITNESSES:

John C. Sanders  
Albert F. Heuman

INVENTOR:

Friedrich Carl Wilhelm Timm  
BY Mr Wallace White

ATTY

# UNITED STATES PATENT OFFICE.

FRIEDRICH CARL WILHELM TIMM, OF HAMBURG, GERMANY.

## PROCESS FOR RECOVERING ZINC FROM ZINKIFEROUS MATERIALS.

1,172,321.

Specification of Letters Patent. Patented Feb. 22, 1916.

Application filed October 7, 1913, Serial No. 793,792. Renewed December 31, 1915. Serial No. 69,684.

To all whom it may concern:

Be it known that I, FRIEDRICH CARL WILHELM TIMM, a subject of the Emperor of Germany, residing at Hamburg, Germany, have invented new and useful Improvements in Processes for Recovering Zinc from Zinkiferous Materials, of which the following is a specification.

This invention relates to a process for blowing zinkiferous materials which contain the zinc in the form of oxid, sulfid, silicate, or other compound, in order to separate and recover the zinc therefrom.

The process consists in blowing the zinkiferous materials, mixed in the known manner with suitable quantities of fuel or reduction material, and (if required by the composition of the zinkiferous materials) some additional materials favoring the reaction as for example lime, oxid of iron, silica and the like. Such additional materials assist in producing either a good sinter, when the pure zinkiferous materials are too strong for sintering or are inclined to smelt at the reaction temperature; or assist in producing a greater yield of zinc, for example by adding a basic substance such as lime instead of another base (zinc oxid) to be driven off. It is known in the art to provide admixtures of appropriate substances to the zinkiferous materials, that are to be deprived of their zinc by ordinary blowing. The blowing consists of treating by means of air or gases containing free oxygen conducted through the charge, thereby producing internal combustion. The said air or gas containing free oxygen is conducted through the charge for a comparatively short time which only suffices for burning a portion of the fuel.

The charge is then removed from the grate or other sustaining device, and is again deposited on the same or another grate or support, and is then again blown and removes as before in such a manner that the blowing is carried out intermittently, to the greatest possible or to the desired degree of dezinkification, on a charge periodically deposited on the grate or support and afterward removed therefrom. The air or other gas used may be conducted through the charge from below upward or in the reverse direction.

The process is intended to overcome the disadvantage, present in the method usually

employed hitherto, of dezinkification by blowing, namely, that owing to the combustion of the fuel the furnace charge shrinks very much and settles irregularly, in consequence of which the gases escape mostly through the gaps, and therefore only pass around the more densely lying portions and there give up their heat less effectually, and drive out the zinc less completely. If, for example, a mixture consisting of two parts by weight of ore and one part of coke breeze is blown in a converter which expands toward the top, then the charge "hangs" in the furnace soon after the "blowing" has commenced. For in this case the relative volumes of ore and coke are about as 1:2, and to this extent therefore there is an empty space above the grate, which space is increased by the sintering of the residue. Owing to the differing sections and the mostly fragmentary to powdery nature of the material to be blown, the sinking down of the charge only takes place irregularly and by fits and starts. In such cases therefore, the higher the charge lies the more unfavorable is the course of the dezinkification. On blowing in a downward direction irregularities in the even distribution of the draft also occur owing to the sinking down of the charge at only some parts of the section, and this effect is more marked the greater the space taken up by the fuel. In working according to the present process, however, the charge is not blown long enough for the empty space arising from the disappearance of the fuel in the zone of combustion to cause any irregular disposition in the rest of the charge, the blowing being interrupted, the charge removed from the grate of the furnace and then deposited anew as regularly as possible on the same or another grate of the same or another furnace, and again blown. The duration and number of repetitions of the blowing are adapted to the nature of the materials to be treated.

It is sometimes specially desirable to make each period of blowing so short that no large compact lumps of sinter are formed. By blowing for only a short period, the hot and soft residue (poor in zinc) of the zone of combustion is broken comparatively easily by removing the charge from the grate; and when mixed with the rest of the

charge may be distributed therein in such a manner that the charge on the grate will have about the same temperature from the top to the bottom and therefore will easily give off the zinc in the next blowing period.

The process may be carried on for example in a converter of the kind illustrated in vertical section in the drawing.

A is the blowing space, B<sub>1</sub>, B<sub>2</sub> the hollow 10 trunnions, C the air admission pipe (stationary), D the gas ejection pipe (stationary), E the opening for charging the heating materials and charge, F the grate, and G a spur-wheel serving for the rotation of 15 the converter by means of gearing.

Red-hot coke is first introduced from above through the opening E on to the grate F. The preferably already preheated charge is then put in, (say previously 20 roasted poor zinc-blende mixed with small coal or coke) and the opening E is closed. By the admission of a small quantity of air the temperature is then so far increased that zinc is evolved from the charge. This zinc 25 passes off with the products of combustion through one of the trunnions, either as vapor, as oxid, or as a mixture of both, according to the purpose required, and to the conditions selected therefor. But after a short 30 time the draft is cut off, and the converter is then turned once or several times about its axis, whereby the contents are mixed up. The same effect may be obtained by an oscillating movement of sufficient amplitude.

35 In order to obtain a layer of even thickness, the movement of the converter is stopped when the surface of its grate has about the same inclination as the angle of repose of the charge in its interior. Then 40 the converter is turned back in the opposite direction until the surface of the charge is evenly distributed over the grate and consequently offers a like resistance to the blast at every part of the grate. It is then again 45 blown for a short time, mixed anew, and these processes are continued alternately until the contents are sufficiently poor in zinc, when they are emptied out through the opening E.

50 Instead of treating a charge as described intermittently in a converter of the kind described or in a similar apparatus by a series of blowing periods and thus decreasing the zinc content from the highest to the lowest

55 grade, the method of working may be made continuous, or approximately continuous, by using a comparatively long converter of the shape of a drum or of a rotary furnace, at one end of which the charge is introduced as 60 regularly as possible, and at the other end of which the dezinkified materials are extracted. The grate in such a long converter extends parallel to the axis and is of fair length but comparatively narrow in width.

65 The charge travels through the converter,

gradually decreasing its zinc content according to its forward movement in the direction of the outlet end, the axis of rotation being arranged at a slight angle as commonly used with rotary furnaces for burning cement 70 and the like. Between every two blowing periods the charge is mixed in itself on account of the rotation then taking place, and at the same time the charge is moved as a whole a little downward, this being caused 75 by the inclination of the furnace. After a certain number of blowing periods, and consequently of revolutions, the material will be moved from the inlet to the outlet and is practically free from zinc. In such a 80 long converter there is always a charge of zinkiferous materials, and it is not necessary to clean it out before a fresh charge is introduced. Further instead of the periodical evolution described the stream of gas and 85 the separation of zinc may be rendered still more continuous, by arranging several grate surfaces on the inner circumferential surface, which on being sufficiently covered with the charge are at the right moment put 90 into connection with the air admission conduit, and disconnected therefrom as soon as (by the rotation or oscillation of the converter) they are no longer sufficiently covered.

95 It may also be mentioned that very fine material may be previously briqueted or made into lumps by some suitable method. In this case larger lumps are preferably made smaller before delivery into the furnace. Further the mixture of the zinkiferous materials with fuel, reduction, and reaction materials may also be made in the furnace, instead of before delivery into it. Further the air, or mixture of gases containing 10 oxygen which serve for blowing is preferably heated.

10 The process renders possible not only the formation of zinc oxid, intelligible without further explanation, which may be separated from the gases in the familiar manner, but also the formation of comparatively pure diluted zinc vapor, if the addition of fuel is made large enough for a complete reduction of the carbon dioxid. This zinc 11 vapor may be recovered by suitable condensation either as metal, as zinc dust, or as oxid by oxidation by the admission of oxygen or in some other form, sulfate for example, by any other suitable subsequent 12 treatment.

12 In this specification the terms "blowing", "to blow", and the like are used as comprehensive terms intended to cover a process for the treatment of materials by means of heat 13 produced internally in the charge to be treated and effecting same by conducting air or other suitable gas under comparatively great difference of pressure through the charge. The difference of pressure be- 130

tween the entering air or gas and exit gas may be obtained either by compressing the air or gas prior to introduction by exhausting the exit gases or by combining both means.

Claims:

1. The process for recovering zinc from zinkiferous materials which consists in causing gas containing free oxygen to pass through a hot mixture of zinkiferous materials and solid carbonaceous substances during a comparatively short time, then withdrawing the mixture from the effect of the gas passing through it, then re-arranging the mixture in a practically even density, then causing the free oxygen containing gas to pass again through the mixture and repeating this working whereby the zinc is freed from the zinkiferous materials in different periods, the heat produced by passing the free oxygen-containing gas through

the mixture being so regulated as to produce an un-molten, sintered residue.

2. The process for recovering zinc from zinkiferous materials which consists in causing air to pass in different periods through a mixture of zinc-containing materials and solid carbon-containing materials, thereby decreasing gradually the zinc content of the charge in different zinc-freeing periods, the charge being between each two such periods remixed in itself and being arranged in a practically even density, the heat being regulated so as to produce a sintered residue.

In testimony whereof I have signed my name to this specification in the presence of two subscribing witnesses.

FRIEDRICH CARL WILHELM TIMM.

Witnesses:

ERNEST H. L. MUMMENHOFF,  
IDA CHRIST. HAERMANN.